

## UNITED STATES PATENT OFFICE

2,081,481

## PROCESS FOR THE PRODUCTION OF NATURAL COLORED IMAGES ON PAPER AND DIAPOSITIVES (CINEMATOGRAPHIC FILMS)

Richard Gschöpf and Karl Pokorny, Vienna, Austria; said Pokorny assignor to said Gschöpf

No. Drawing. Application January 10, 1934,  
Serial No. 706,128. In Austria July 22, 1933

6 Claims. (Cl. 101—149)

This invention relates to the production of colored prints, and natural colored images on paper and diapositives (cinematographic films).

A number of processes are known for the production of natural colored prints.

Apart from the colored pictures (autochromatic prints) obtained with screen elements (additive methods) there are only the subtractive methods available for the production of natural 10 colored prints.

In the latter methods gelatine printing matrices (swelling and washing out relief) are as a rule produced from the three component negatives, and these matrices have hitherto been 15 colored with the normal commercial acid and basic dyes, and then squeegeed one upon the other onto a common image carrier coated with gelatine.

The acid dyes pass over imperfectly and also 20 very slowly from the gelatine printing matrices to the image carrier. This involves great drawbacks, the obviation of which has been attempted by the employment of basic dyes.

The basic dye-stuffs pass over rapidly from 25 the gelatine printing matrix (relief) to the image carrier. However, they are apt to run and spread in the gelatine layer of the latter.

However, if image carriers be employed the 30 gelatine layer of which is provided with precipitants for these dyestuffs, the matrices "bleed", that is to say they part with the absorbed coloring matter so rapidly during the squeegeeing onto the image carrier, that it forms on the entire surface of the latter a thin insoluble dye 35 compound which also tones the colorless portions (the whites) of the picture, thus smudging these portions.

There are only very few dyes, such as fuchsin (magenta) which do not bleed out. These dyes, 40 however, do not pass over perfectly onto the image carrier. The chemical combining of the dye in the gelatine printing matrix and the subsequent liberation of the same does not lead to satisfactory results either.

A satisfactory result can, therefore, only be 45 achieved provided the coloring matter be so firmly incorporated or lodged, not chemically but physically, in the gelatine printing matrix, 50 that no "bleeding" out of this matter occurs.

According to most recent knowledge, an important part is played in connection with the coloring of gelatine with dyestuff by the chemical process (cf. report on paper read by E. R. Bullock to the Faraday Society, given in "The

Physical Chemistry of the Photographic Process", May, 1923, pages 396-401).

By effecting chemical combining of the dye in the gelatine of the printing matrix, the arbitrariness of the absorption and giving up of the 5 color is not overcome, and all that is actually effected is to render the yielding up of the coloring matter more difficult than otherwise. But also the chemical process occurring in the course of color transference points to the fact that the 10 basic dyes are unsuitable as such for the production of colored pictures. The base of the dye combines with the mordant or precipitant used (silicotungstic acid, phosphotungstic acid, or the like) as an ingredient of the material of the image carrier, while the liberated acid of the basic 15 dye exerts a deleterious influence on the matrix by imparting acid character to the gelatine layer which tends to counteract all further coloration.

Finally, such dye becomes most firmly anchored in the colloidal structure of the gelatine 20 as is of a molecular size suited to this structure.

It will be clear from what has been said above that firm adherence of the dye to the gelatine 25 of the matrix, without chemical combining, can only be attained if the dye be in colloidal solution, be freed from acid, and be caused to be of a molecular size best suited for coloration; that is to say if pure dye bases be employed for the coloration.

With the employment of this variety of the 30 usual basic dyes it is a simple matter to avoid all the drawbacks attendant upon the use of the two other varieties.

Thus in accordance with the invention, instead of sulphuric acid, hydrochloric acid, acetic acid and other salts of dye bases, there are employed colloidal solutions of dye bases for the coloration of the matrices (reliefs).

These solutions have the property of adhering 35 relatively firmly to the gelatine relief, and that without chemical combining, and nevertheless of passing over extremely rapidly (given suitable treatment of the image carrier in some seconds) and perfectly quantitatively, that is to say without remainder, into the image carrier provided with precipitants.

The preparation of the colloidal dye bases in 40 solution is extremely simple; a suitably concentrated dye solution of the basic dye-stuff concerned, for example thionine blue, is prepared, and to this there is added, for example, ammonia in such quantity and until the solution is of 45 strongly alkaline reaction, that is to say until the dye base has been liberated.

However, there also exist basic dye-stuffs the colloidal dye base solutions of which produced with ammonia begin to separate out in a comparatively short time in the form of a flocculent precipitate, and which are consequently unsuitable for the coloring of gelatine reliefs when merely used in this manner.

Now this can be prevented by adding pyridine, its derivatives, and homologues to the dye-stuff solution or to the colloidal dye base solution produced by the addition of ammonia.

Whether the pyridine or substances of a pyridine-like nature form complex compounds with the colloidal solutions of dye bases is in this connection of subsidiary importance. It is a fact that an addition of pyridine results in perfectly clear solutions of a colloidal nature of the majority of dye bases, which solutions do not yield flocculent precipitates.

20. In the case of basic dye-stuffs of which the colloidal dye base solutions yield flocculent precipitates even with the treatment specified above, it is further necessary to add to the solutions certain protective colloids such as dextrine and 25 the like, and to remove the salts, such as ammonium nitrate, ammonium sulphate, and the like formed by the alkalies, by dialysis.

For example, in order to obtain a free dye base of new solid green which does not flock out, 30 there is added to a solution (of approximately 1% strength) of this dye-stuff, approximately 0.1% of dextrine as a protective agent, and ap-

proximately 1 ccm. of pyridine, after which this solution is then treated as specified above.

Where intensification of the alkaline reaction is desired, it is apparent that a substance of alkaline reaction may be added to the colloidal solutions of the dye bases, if desired.

We claim:

1. A process for the production of single and multicolored prints, consisting in coloring photographic gelatine printing matrices by means of 10 colloidal solutions of dye bases, and transferring the absorbed dye base to a carrier provided with precipitants.

2. A process as defined in claim 1, wherein a substance of alkaline reaction is added to the 15 colloidal solutions of the dye bases for intensifying the alkaline reaction.

3. A process as defined in claim 1, wherein the 20 colloidal solutions of dye bases are produced with the aid of pyridine.

4. A process as defined in claim 1, wherein protective colloids are added in small quantities to the colloidal solutions of the dye bases.

5. A process as defined in claim 1, wherein the 25 colloidal solutions of dye bases are produced with the aid of derivatives of pyridine.

6. A process as defined in claim 1, wherein the 30 colloidal solutions of dye bases are produced with the aid of homologues of pyridine.

RICHARD GSCHÖPF.  
KARL POKORNY.

20

30